

March 28, 1950

G. V. SLOTTMAN

2,502,284

DECARBURIZATION OF STEEL

Filed Nov. 22, 1947

2 Sheets-Sheet 1



FIG. 1

INVENTOR  
GEORGE V. SLOTTMAN  
BY

*Perkins, Edmund, Norton & Bassett*  
ATTORNEYS

March 28, 1950

G. V. SLOTTMAN  
DECARBURIZATION OF STEEL

2,502,284

Filed Nov. 22, 1947

2 Sheets-Sheet 2



FIG. 2



FIG. 3

INVENTOR  
GEORGE V. SLOTTMAN  
BY  
*Perkins, Polk & Mohr, Barron*  
ATTORNEYS

## UNITED STATES PATENT OFFICE

2,502,284

## DECARBURIZATION OF STEEL

George V. Slottman, New York, N. Y., assignor to  
 Air Reduction Company, Incorporated, New  
 York, N. Y., a corporation of New York

Application November 22, 1947, Serial No. 737,488

3 Claims. (Cl. 75—60)

**1**

This invention relates to the manufacture of steel and particularly to the elimination of excess carbon from the steel during production thereof.

In an application Ser. No. 728,868, I have described a method of producing steel in an open hearth furnace in which, after the steel has reached the point of decarburization, oxygen is introduced through a pipe to burn and thus eliminate the excess carbon. The oxygen disseminates through the molten metal rapidly and is startlingly efficient as a decarburizer until the carbon content falls below 0.25%. Thereafter the effectiveness of the oxygen decreases rapidly until, in the region of .03% carbon, the efficiency is only about 5%. This is readily understood because the molten metal consists of a shallow layer only about 25 inches deep in a surface area in the vicinity of 600 square feet. The oxygen must diffuse through distances of up to 20 feet and therefore much of it is lost during the latest stages of the reaction, by combination with iron and in the overlying slag layer. While no difficulty is experienced in the early stages of decarburization because the oxygen disseminates rapidly, as is evidenced by carbon monoxide flames over the entire surface of the metal, it is relatively difficult to bring the carbon content below 0.25% by the method as heretofore practiced.

It is the object of the present invention to provide a method of applying oxygen more effectively in the decarburizing of steel, whereby the difficulties mentioned are overcome and the oxygen is efficient even after the carbon content is below 0.25% in the molten metal.

Other objects and advantages of the invention will be apparent as it is better understood by reference to the following specification and the accompanying drawings, in which

Fig. 1 is a diagrammatic illustration of an apparatus suitable for the practice of the invention;

Fig. 2 is a modified form of such apparatus; and

Fig. 3 illustrates another modified form of the apparatus.

In accordance with the present invention, the production of steel may be carried out in an open hearth or other suitable furnace. In an open hearth furnace, selected scrap is first melted on the hearth and, when melting is completed, suitable additions are made in accordance with the usual practice. The heat is continued until analysis of the metal indicates that the composition is satisfactory except for the excess carbon content which is always present in steel produced in

**2**

the manner described and particularly in open hearth practice.

At this point, the furnace is tapped and the metal is withdrawn. Oxygen is introduced to the metal for the purpose of eliminating the excess carbon and bringing the carbon content down to the required percentage for the particular purpose for which the metal is intended. Introduction of oxygen may be accomplished in a variety of ways. In one embodiment of the invention, a holding receptacle is provided, through which the molten metal flows continuously while oxygen is introduced to the flowing metal. Instead of introducing the oxygen in a holding receptacle, it may be directed into the flowing stream of metal leaving the furnace. Or, the molten metal may be delivered to a relatively large receptacle of substantial depth compared with its cross-sectional area, and oxygen may be introduced to the molten metal until a satisfactory composition is attained. Thereafter the completed metal heat may be delivered to a receptacle for transportation such as a ladle. In each of the cases mentioned, the molten metal is subjected to the action of sufficient oxygen to consume the excess carbon and bring the carbon content to the required percentage. Since the metal is no longer in the form of a shallow layer as on the hearth of the open hearth furnace, there is no problem of dissemination of the oxygen. All of the metal is subjected uniformly to the action of oxygen which reacts actively with the carbon present, and the desired result is readily attained.

Although oxygen of commercial purity, that is 35 99.5% or better is most suitable for the purpose, it is not essential. Oxygen of purity range from 45% to 99.5% or better may be utilized successfully for the purpose of the present invention. The reaction is slower with lower grades of oxygen, but nevertheless the carbon may be consumed effectively and more satisfactorily with respect to certainty of results than by the method as heretofore commonly practiced, in which iron ore is added as an oxidizing agent to eliminate 45 carbon.

Referring to the drawing, 5 indicates an open hearth furnace having a hearth 6, a charging opening 7 and a tapping hole 8. Scrap steel may be melted on the hearth 6 in the usual manner 50 with suitable additions of lime to form a slag and of blast furnace iron to provide the molten steel 9 and its overlying layer of slag 10. Heat is supplied in the usual manner by burners (not shown) at the ends of the furnace. The details 55 of the furnace structure form no part of the

present invention, and since such furnaces are in common use, further description is unnecessary.

When the heat is completed, except for the presence of excess carbon, the molten metal is tapped through the tapping hole 8 and is delivered by a runner 11 to a receptacle 12 of suitable heat resistant construction, affording a relatively deep space as compared with the cross-sectional area. The receptacle 12 has an outlet 13 through which the metal flows, by means of a runner 14, into a ladle 15. The apparatus is proportioned so that the flow of molten metal is continuous, that is, the amount flowing into the receptacle 12 is continuously withdrawn through the outlet 13. While the molten metal is in the receptacle 12, it is subjected to the action of oxygen supplied through a tuyère 16 which is connected by a pipe 17 to a source of oxygen under suitable pressure. Thus the oxygen bubbles up through the molten metal, and the carbon content is rapidly oxidized and thus eliminated. The molten metal flowing into the ladle 15 will have a predetermined carbon content, the operation being regulated in view of the proportion of carbon present in the molten steel as it leaves the furnace 5. More or less oxygen may be supplied as required to accomplish the intended purpose.

Referring to Fig. 2 of the drawing, a furnace 18, for example of the open hearth type having a hearth 19, charging openings 20 and a tapping hole 21, is operated in the manner hereinbefore described until the steel has the required composition except for excess carbon. The furnace is then tapped, and the molten metal is delivered through a runner 22 into a ladle 23. A pipe 24 is disposed so that it discharges oxygen into the flowing stream of molten metal in the runner 22. The pipe 24 may be connected to a source of oxygen under suitable pressure. Thus, all of the metal flowing from the furnace is subjected to the action of oxygen, which reacts with the carbon in the metal during transit through the runner 22 and in the ladle 23. The excess carbon is thus eliminated to the desired point to produce steel of the required carbon composition.

In Fig. 3, a furnace 25 has a tapping hole 26 and the molten metal 27 therein, after reaching a suitable composition except for excess carbon, is delivered through a runner 28 to a receptacle 29 which is relatively deep as compared with its cross-sectional area, and adapted to hold the entire heat or a part of the heat from the furnace 25. A pipe 30 extends into the receptacle 29 and encloses an inner pipe 31 through which oxygen is supplied from any suitable source. A coolant may be delivered to the pipe 30 from a source 32 and withdrawn through a pipe 33, so that the pipe 30 and the pipe 31 will not be consumed. The oxygen is delivered to the molten metal which is held in considerable depth and the carbon is readily consumed so that a metal of the desired carbon composition is easily obtainable. In each of the cases described, the difficulty arising through the necessity for disseminating oxygen through a shallow layer of molten metal in the open hearth furnace is eliminated. Where there is a considerable depth of metal, the oxygen, having a tendency to rise to the surface, thoroughly impregnates all of the metal and comes into contact with the carbon which it oxidizes.

Various changes may be made in the procedure

as described without departing from the invention or sacrificing the advantages thereof.

I claim:

- 5 1. The method of decarburizing steel which comprises subjecting it in a molten state in an open hearth furnace to an initial refining operation with reduction of the carbon content thereof to about 0.25%, withdrawing the initially decarburized steel in a molten state from the furnace, maintaining the withdrawn steel in a molten state, and forming a flowing body of the initially decarburized and molten steel which is relatively deep with respect to its cross-sectional area, and thereafter introducing a gas containing more than 45% oxygen into the lower portion of said relatively deep body of molten steel until it has reacted with the carbon content of the molten steel sufficiently to bring about a further substantial reduction of the carbon content thereof.
- 10 2. The method of decarburizing steel which comprises subjecting it in a molten state in an open hearth furnace to an initial refining operation with reduction of the carbon content thereof to about 0.25%, withdrawing the initially decarburized steel in a molten state from the furnace, maintaining the withdrawn steel in a molten state, flowing the withdrawn molten steel past a source of a gas containing more than 45% oxygen, and introducing gas from said source into the flowing stream and reacting the oxygen content thereof with the carbon of the flowing molten steel in amount sufficient to substantially further reduce the carbon content thereof.
- 15 3. The method of decarburizing steel which comprises subjecting it in a molten state in an open hearth furnace to an initial refining operation with reduction of the carbon content thereof to about 0.25%, withdrawing the initially decarburized steel in a molten state from the furnace, maintaining the withdrawn steel in a molten state, and forming a body of the initially decarburized and molten steel which is relatively deep with respect to its cross-sectional area, and thereafter introducing a gas containing more than 45% oxygen into the lower portion of said relatively deep body of molten steel until it has reacted with the carbon content of the molten steel sufficiently to bring about a further substantial reduction of the carbon content of the molten steel.

GEORGE V. SLOTTMAN.

#### REFERENCES CITED

- 55 The following references are of record in the file of this patent:

#### UNITED STATES PATENTS

|    | Number    | Name       | Date          |
|----|-----------|------------|---------------|
| 60 | 16,690    | Martien    | Feb. 24, 1857 |
|    | 465,672   | Lindenthal | Dec. 22, 1891 |
|    | 1,133,317 | Rice       | Mar. 30, 1915 |
|    | 1,312,474 | Fisk       | Aug. 5, 1919  |
|    | 1,394,103 | McGlynn    | Oct. 18, 1921 |
| 65 | 1,484,465 | Billings   | Feb. 19, 1924 |
|    | 1,756,054 | Crum       | Apr. 29, 1930 |
|    | 2,074,164 | Clair      | Mar. 16, 1937 |

#### FOREIGN PATENTS

|    | Number  | Country       | Date         |
|----|---------|---------------|--------------|
| 70 | 12,356  | Great Britain | of 1886      |
|    | 20,245  | Great Britain | of 1902      |
|    | 156,548 | Great Britain | Apr. 5, 1922 |